



US006436619B1

(12) **United States Patent**  
Majumdar et al.

(10) **Patent No.:** US 6,436,619 B1  
(45) **Date of Patent:** Aug. 20, 2002

(54) **CONDUCTIVE AND ROUGHENING LAYER**

(75) Inventors: **Debasis Majumdar**, Rochester;  
**Thomas M. Laney**, Spencerport;  
**Jehuda Greener**, Rochester; **Jose L. Garcia**, Webster; **Peter T. Aylward**, Hilton, all of NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/853,846**

(22) Filed: **May 11, 2001**

(51) **Int. Cl.**<sup>7</sup> ..... G03C 1/765; G03C 1/89

(52) **U.S. Cl.** ..... **430/496**; 430/527; 430/528;  
430/531; 430/533; 430/536

(58) **Field of Search** ..... 430/527, 528,  
430/496, 523, 531, 533, 536

(56)

**References Cited**

**U.S. PATENT DOCUMENTS**

|              |        |                        |         |
|--------------|--------|------------------------|---------|
| 5,902,720 A  | 5/1999 | Haydock et al. ....    | 430/536 |
| 6,022,677 A  | 2/2000 | Bourdelaix et al. .... | 430/536 |
| 6,030,742 A  | 2/2000 | Bourdelaix et al. .... | 430/536 |
| 6,197,486 B1 | 3/2001 | Majumdar et al. ....   | 430/527 |
| 6,207,361 B1 | 3/2001 | Greener et al. ....    | 430/527 |

*Primary Examiner*—Richard L. Schilling

(74) *Attorney, Agent, or Firm*—Paul A. Leipold; Lynne M. Blank

(57) **ABSTRACT**

The invention relates to a material comprising a web wherein said web comprises at least one surface layer comprising polyether polymeric antistat, extrudable polymer, and compatibilizer wherein said surface layer has a roughness of greater than 0.3 Ra.

**22 Claims, No Drawings**

## CONDUCTIVE AND ROUGHENING LAYER

## FIELD OF THE INVENTION

This invention relates to a conductive and roughening layer. In a preferred form it relates to imaging elements, particularly laminated base materials for imaging elements.

## BACKGROUND OF THE INVENTION

The problem of controlling static charge during plastic web manufacturing and transport is well known. Generation and uncontrolled discharge of electrostatic charge can cause a number of serious problems including safety hazards. In the field of imaging, particularly photography, the accumulation of charge on film or paper surfaces leads to the attraction of dirt, which can produce physical defects. The discharge of accumulated charge during or after the application of the sensitized emulsion layer(s) can produce irregular fog patterns or "static marks" in the emulsion. The static problems have been aggravated by increase in the sensitivity of new emulsions, increase in coating machine speeds, and increase in post-coating drying efficiency. The charge generated during the coating process may accumulate during winding and unwinding operations, during transport through the coating machines and during finishing operations such as slitting and spooling.

It is generally known that electrostatic charge can be dissipated effectively by incorporating one or more electrically-conductive "antistatic" layers into the support structure. Typical location of an antistatic layer is an external surface, which comes in contact with various transport rollers. For imaging elements, the antistatic layer is usually placed on the side of the support opposite to the imaging layer.

A wide variety of electrically-conductive materials can be incorporated into antistatic layers to produce a wide range of conductivities. These can be divided into two broad groups: (i) ionic conductors and (ii) electronic conductors. In ionic conductors charge is transferred by the bulk diffusion of charged species through an electrolyte. Here the resistivity of the antistatic layer is dependent on temperature and humidity. Antistatic layers containing simple inorganic salts, alkali metal salts of surfactants, ionic conductive polymers, polymeric electrolytes containing alkali metal salts, and colloidal metal oxide sols (stabilized by metal salts), described previously in patent literature, fall in this category. However, many of the inorganic salts, polymeric electrolytes, and low molecular weight surfactants used are water-soluble and are leached out of the antistatic layers during processing, resulting in a loss of antistatic function. The conductivity of antistatic layers employing an electronic conductor depends on electronic mobility rather than ionic mobility and is independent of humidity. Antistatic layers which contain conjugated polymers, semiconductive metal halide salts, semiconductive metal oxide particles, etc., have been described previously. However, these antistatic layers typically contain a high volume percentage of electronically conducting materials, which are often expensive and impart unfavorable physical characteristics, such as color, increased brittleness and poor adhesion, to the antistatic layer.

A vast majority of the prior art involves coatings of antistatic layers from aqueous or organic solvent based coating compositions. For photographic paper, typically antistatic layers based on ionic conductors, are coated out of aqueous and/or organic solvent based formulations, which necessitate an effective elimination of the solvent. Under fast drying conditions, as dictated by efficiency, formation of

such layers may pose some problems. An improper drying will invariably cause coating defects and inadequate adhesion and/or cohesion of the antistatic layer, generating waste or inferior performance. Poor adhesion or cohesion of the antistatic layer can lead to unacceptable dusting and track-off. A discontinuous antistatic layer, resulting from dusting, flaking, or other causes, may exhibit poor conductivity, and may not provide necessary static protection. It can also allow leaching of calcium stearate from the paper support into the processing tanks causing build-up of stearate sludge. Flakes of the antistatic backing in the processing solution can form soft tar-like species, which, even in extremely small amounts, can re-deposit as smudges on drier rollers eventually transferring to image areas of the photographic paper, creating unacceptable defects.

Moreover, majority of antistats on current photographic paper products lose their electrical conductivity after photographic processing due to their ionic nature. This can cause print sticking after drying in the photoprocessor, and/or in a stack.

In U.S. Pat. Nos. 6,197,486 and 6,207,361, antistatic layers have been disclosed which can be formed through the (co)-extrusion method thus eliminating the need to coat the support in a separate step and rendering the manufacturing process less costly.

When placed as an external layer, the antistatic layer may be required to fulfill additional criteria depending on the application. One such criterion is the conveyance of the web through many different types of equipment. For photographic paper, for example, the web must convey through various machines, which involve base making, sensitizing, slitting, photographic printing, processing, finishing, etc. Efficient transport of such products necessitates a tight control of the roughness of the external layer. As disclosed in U.S. Pat. No. 6,022,677, photographic papers with a backside roughness average,  $R_a$ , of less than  $0.3 \mu\text{m}$  cannot be efficiently transported in the photoprocessing equipment, as many transport problems will occur. Transport problems such as, scratching, machine jams, and poor print sticking will occur with backside  $R_a$  of less than  $0.3 \mu\text{m}$ . In majority of color paper products, such a desirable roughness on the backside of the paper can be achieved by casting polyethylene against a rough chilled roll. Photographic papers made in this manner are very efficiently transported through photoprocessing equipment. However, polyethylene coated photographic papers, when exposed to varying humidity, may experience serious curl that can interfere with the viewing of images. A solution to this curl problem is proposed in U.S. Pat. No. 5,902,720, through the use of biaxially oriented polyolefin sheets, which unfortunately provides a backside roughness of  $R_a$  less than  $0.23 \mu\text{m}$ .

In the final image format, it is common for consumers to write personal information on the backside of the images with pens, pencils, and other writing instruments. Photographic papers that are smooth on the backside are more difficult to write on. There is also a desire to print information from Advanced Photo System negatives onto prints made from these negatives. Therefore, there is a need for color prints to receive printing and writing on their back. There remains a need for photographic papers that are sufficiently rough so that writing or printing on the backside of the photographs can be easily accomplished.

During the manufacturing process for photographic papers, it is a requirement that silver halide emulsion coated paper be handled and transported in roll form. In roll form, the backside of the photographic paper is in contact with the

silver halide image forming layer. If the roughness of the backside exceeds 2.54  $\mu\text{m}$ , the image forming layer would begin to become embossed with the surface roughness pattern while in the roll form. Any customer perceived embossing of the image forming layer will significantly decrease the commercial value of the image forming layer. Furthermore, silver halide emulsions tend to be pressure sensitive. A sufficiently rough backside, in roll form, would begin to also destroy the commercial value of the image forming layer by developing the silver emulsion with pressure from the surface roughness of the backside. There remains a need for a photographic paper that has a backside roughness less than 2.54  $\mu\text{m}$  so that photographic paper can be conveniently wound and stored in roll format.

In the formation of reflective receivers for digital imaging systems such as Ink Jet and Thermal Dye Transfer, there is a need to reduce the curl of the image. Lamination of a high strength biaxially oriented polyolefin sheet to the backside of the image does improve the curl over the common practice of extrusion coating a layer of polyolefin. Reflective receivers for digital imaging systems that have a smooth backside will cause transport problems in the various types of printers that are common in digital printing. Transport difficulties resulting from a smooth backside could cause unacceptable paper path jams, scratches on the image, and failure to pick the receiver from a stack. The latter problem can be further aggravated by electrostatic attraction between contiguous sheets. For ink jet and thermal dye transfer receivers it would be desirable if a backside surface could be formed with a surface roughness greater than 0.30  $\mu\text{m}$  with antistatic characteristics to allow for efficient photoprocessing.

Photographic papers with biaxially oriented polyolefin sheets with a backside Ra between 0.3  $\mu\text{m}$  and 2.0  $\mu\text{m}$  are proposed in U.S. Pat. Nos. 6,022,677 and 6,030,742. The roughness of the backside surface is claimed to have been achieved either through the use of particulate addenda or by a mixture of incompatible block copolymers of polyethylene and polypropylene. Although these polyolefin sheets possess the desired roughness, they lack electrical conductivity, and therefore require separate antistatic layers for effective charge control.

#### PROBLEM TO BE SOLVED BY THE INVENTION

There remains a need for materials comprising a web wherein the surface of the web is electrically conducting and has a roughness between 0.3  $\mu\text{m}$  and 2.0  $\mu\text{m}$  Ra, which, if incorporated in an imaging element, will provide antistatic characteristics, easy conveyance and efficient photoprocessing, storage without blocking and backside writability and printability.

#### SUMMARY OF THE INVENTION

It is an object of the invention to provide materials comprising a web wherein the surface of the web is electrically conducting.

It is another object to provide the aforesaid surface with desirable roughness characteristics.

It is a further object to provide improved imaging elements with an antistatic surface and desirable roughness characteristics, which can be efficiently conveyed during manufacturing, sensitizing, finishing and processing, and can be easily written or printed on.

These and other objects of the invention are accomplished by a material comprising a web wherein said web comprises

at least one surface layer comprising polyether polymeric antistat, extrudable polymer, and compatibilizer wherein said surface layer has a roughness of greater than 0.3 Ra.

#### ADVANTAGEOUS EFFECT OF THE INVENTION

The invention provides improved web based materials, which are antistatic. The invention also provides desirable roughness characteristics to the web surface for easy conveyance during various phases of manufacturing and processing. The invention further provides backside writability and printability. Moreover, the web of the invention can be formed through thermal processing, such as extrusion and co-extrusion, without solvent based coating.

#### DETAILED DESCRIPTION OF THE INVENTION

There are numerous advantages of the invention over prior practices in the art. The invention provides improved web based materials, which are antistatic. When implemented in an imaging element, particularly photographic products, the invention provides antistatic characteristics before and after photographic processing. The surprising characteristic of post-processing conductivity in the web of the invention, can minimize print sticking, dirt attraction, and other problems commonly encountered in photographic products.

The invention also provides a web surface with the roughness characteristics desirable for easy conveyance. When incorporated on the backside of photographic products, the invention allows for efficient transport through photoprocessing equipment. Photographic papers with a smooth back surface can experience transport difficulties and jamming in machines required for developing, transporting and packaging of photographic paper.

Another advantage of the invention is realized during the end-use by the customer. Images in the final customer format are commonly stored on top of each other. In this format, the backside of the photographic image is placed in contact with the emulsion side, and there is a tendency for the images to stick together. Sticking can be aggravated both under dry conditions, due to generation of static charge, and under hot and humid conditions, due to the tackiness of the image layer. Such sticking makes subsequent handling of the stacked images difficult, as the consumer must separate the images. The invention, through its control of backside roughness and antistatic characteristics, minimizes the tendency of image sticking for the customer.

A further advantage of this invention is a more effective surface for writing and printing on the backside of images. The ability to write on the backside images using conventional writing instruments such as pens and pencils is a function of both surface roughness and ability of the surface to absorb inks. The invention also allows for faster printing of Advanced Photo System information. This invention allows for increasing surface roughness and, thus, the ability for the consumer or printer to write necessary information on the backside of the image.

Another advantage of this invention is the ability to more efficiently create roughness on the backside of the images. Prior practices utilized expensive coatings that, when dry, increase the roughness of the backside. Prior practices also utilized the casting of the backside polyethylene against expensive rough chilled rolls to create the surface roughness for effective conveyance, however, without good writability with something as common as a pencil.

Yet another advantage of this invention is the dual characteristics of the web of the invention provide conductivity and roughness through a single layer. In prior art, particularly for photographic paper, a backside roughness of  $0.3 \mu\text{m}$  and  $2.0 \mu\text{m}$  Ra is typically generated in the resin layer by some suitable means, which is subsequently coated with an overlying thin antistatic layer that essentially maintains the roughness characteristics. In such two-step processes, the speed of manufacturing is typically limited by the speed at which the antistatic layer can be coated and dried on the resin. The present invention eliminates the two-step process and provides a resin layer that is both rough and antistatic, which can be applied to any substrate, for example photographic paper, at a much faster speed than solvent based coatings. These and other advantages of the invention will be apparent from the detailed description below.

The terms as used herein, "top", "upper", "emulsion side", and "face" mean the side or toward the side of the imaging member bearing the imaging layers. The terms "bottom", "lower side", and "back" mean the side or toward the side of the imaging member opposite from the side bearing the imaging layers or image. The term "void" as used in "voided polymer" is used herein to mean devoid of added solid or liquid matter, although it is likely the "voids" contain gas. The term "voided polymers" will include materials comprising polymeric foam, microvoided polymers and microporous materials known in the art.

The surface layer of the web of the invention comprises polyether polymeric antistat as component A, extrudable polymer as component B, and compatibilizer as component C.

Polyether based polymeric antistats (Component A) are suitable materials containing polyalkoxylated compounds, which are well known in the art for their excellent melt-processability while retaining their antistatic property and overall physical performance. These materials can include various polymeric substances containing polyether blocks such as polyethylene oxides, polypropylene oxides, polybutylene oxides, polytetramethylene oxides, polyoxylakylene glycols such as polyoxyethylene glycol, polyoxypropylene glycol, polyoxytetramethylene glycol, the reaction products of polyalkoxylates with fatty acids, the reaction products of polyalkoxylates with fatty alcohols, the reaction products of polyalkoxylates with fatty acid esters of polyhydroxyl alcohols (for instance polyalkoxylate reaction products of fatty acids, of fatty glycols, of fatty sorbitols, of fatty sorbitans, and of fatty alcohols), or, interpolymers and/or mixtures thereof. The polyether chains in the suitable polyalkoxylated compounds are of the formula  $(-\text{OC}_x\text{H}_{2x}-)_n$  wherein x is from 2 to about 8, wherein the alkyl group is straight or branched, and wherein n is from 2 to about 1000. It is believed that ionic conduction along the polyether chains makes these polymers inherently dissipative, yielding surface resistivities in the range  $10^8$ – $10^{13}$  ohm/square. For the purpose of this invention any polyalkoxylated compounds containing oligomer, homopolymer, interpolymer and/or mixtures thereof can suitably be used as component A in this invention. However, preferred examples of such polyether polymeric antistatic materials are: those comprising polyamide blocks and polyether block(s), e.g., as disclosed in U.S. Pat. Nos. 4,331,786, 4,115,475, 4,195,015, 4,839,441, 4,864,014, 4,230,838 and 4,332,920 and product literature for Pebax supplied by Elf Atochem, polyetheresteramides, e.g., as disclosed in U.S. Pat. Nos. 5,604,284; 5,652,326; 5,886,098, and thermoplastic polyurethanes containing a polyalkylene glycol moiety, e.g., as disclosed in U.S. Pat. Nos. 5,159,053; 5,863,466, with the content of all of the

aforementioned literature incorporated herein by reference. Most preferred polyether polymeric antistats are those comprising polyamide blocks and polyether block(s).

Polymers comprising polyamide blocks and polyether block(s) result from the copolycondensation of polyamide sequences containing reactive ends with polyether sequences containing reactive ends, such as, inter alia: 1) Polyamide sequences containing diamine chain ends with polyoxylakylene sequences containing dicarboxyl chain ends, 2) Polyamide sequences containing dicarboxyl chain ends with polyoxylakylene sequences containing diamine chain ends obtained by cyanoethylation and hydrogenation of alpha.,omega.-dihydroxylated aliphatic polyoxylakylene sequences known as polyetherdiols, 3) Polyamide sequences containing dicarboxyl chain ends with polyetherdiols, the products obtained being, in this specific case, polyetheresteramides.

The polyamide sequences containing dicarboxyl chain ends result, for example, from the condensation of alpha.,omega.-aminocarboxylic acids from lactams or of dicarboxylic acids and diamines in the presence of a chain-limiting dicarboxylic acid. The polyamide blocks are advantageously formed from polyamide-6/12.

The number-average molecular mass or weight Mn of the polyamide sequences is between 300 and 15,000 and preferably between 600 and 5,000. The Mn of the polyether sequences is between 100 and 6,000 and preferably between 200 and 3,000.

The polymers containing polyamide blocks and polyether blocks can also comprise units distributed randomly. These polymers can be prepared by the simultaneous reaction of the polyether and the precursors of the polyamide blocks.

For example, polyetherdiol, a lactam (or an alpha.,omega.-amino acid) and a chain-limiting diacid can be reacted in the presence of a small amount of water. A polymer is obtained having essentially polyether blocks and polyamide blocks of highly variable length but also the various reactants, which have reacted randomly, distributed statistically along the polymer chain.

These polymers contain polyamide blocks and polyether blocks, whether they originate from the copolycondensation of polyamide and polyether sequences prepared beforehand or from a single-stage reaction, exhibit, for example, Shore D hardnesses which can be between 20 and 75 and advantageously between 30 and 70 and an intrinsic viscosity between 0.8 and 2.5, measured in metacresol at  $25^\circ\text{C}$ .

Whether the polyether blocks derive from polyethylene glycol, from polypropylene glycol or from polytetramethylene glycol, they are either used as they are and copolycondensed with polyamide blocks containing carboxyl ends or they are aminated in order to be converted to polyetherdiamines and condensed with polyamide blocks containing carboxyl ends. They can also be mixed with polyamide precursors and a chain limiter in order to prepare polymers containing polyamide blocks and polyether blocks having units distributed statistically.

The polyether can be, for example, a polyethylene glycol (PEG), a polypropylene glycol (PPG) or a polytetramethylene glycol (PTMG). The latter is also known as polytetrahydrofuran (PTHF).

Whether the polyether blocks are introduced into the chain of the polymer containing polyamide blocks and polyether blocks in the form of diols or diamines, they are known for simplicity as PEG blocks or PPG blocks or alternatively PTMG blocks. It would not be departing from the scope of the invention if the polyether blocks contained

different units, such as units derived from ethylene glycol, from propylene glycol or alternatively from tetramethylene glycol.

The polyamide blocks typically comprise condensation product of: one or a number of amino acids, such as aminocaproic, 7-aminoheptanoic, 11-aminoundecanoic and 12-aminododecanoic acids, or one or a number of lactams, such as caprolactam, oenantholactam and lauryllactam; one or a number of salts or mixtures of diamines, such as hexamethylenediamine, dodecamethylenediamine, meta-xylylenediamine, bis-(*p*-aminocyclohexyl)methane and trimethylhexamethylene-diamine, with diacids, such as isophthalic, terephthalic, adipic, azelaic, suberic, sebacic and dodecanedicarboxylic acids; or mixtures of some of these monomers, which result in copolyamides, for example polyamide-6/12 (or nylon-6/12) by condensation of caprolactam and lauryllactam. Polyamide mixtures can be used.

Preferably, the polymer having polyamide blocks and polyether blocks comprises a single type of block. Advantageously, polymers having polyamide-12 blocks and PEG blocks, and polymers having polyamide-6 blocks and PEG blocks are employed. One can however also employ blends of polymers having polyamide blocks and polyether blocks.

Polymers containing polyamide blocks and polyether blocks particularly useful for this invention are described in U.S. Pat. Nos. 4,331,786; 4,115,475; 4,195,015; 4,839,441; 4,864,0143; 4,230,838 and 4,332,920. Such polymers include products such as Pebax, available from Elf Atochem or similar materials. These types of polyether antistatic polymers have been shown to be fairly thermally stable and readily processable in the melt state in their neat form or in blends with other polymeric materials.

The extrudable polymer (component B) of the invention can be any suitable thermoplastic polymer. Suitable classes of thermoplastic polymers preferred for this invention can include polymers of alpha-beta unsaturated monomers, polyesters, polyamides, polycarbonates, cellulosic esters, polyvinyl resins, polysulfonamides, polyethers, polyimides, polyurethanes, polyphenylenesulfides, polytetrafluoroethylene, polyacetals, polysulfonates, polyester ionomers, and polyolefin ionomers. Interpolymers and/or mixtures of these polymers can also be used.

Illustrative of polymers of alpha-beta unsaturated monomers, which are suitable for use in this invention include polymers of ethylene, propylene, hexene, butene, octene, vinylalcohol, acrylonitrile, vinylidene halide, salts of acrylic acid, salts of methacrylic acid, tetrafluoroethylene, chlorotrifluoroethylene, vinyl chloride, styrene and the like. Interpolymers and/or mixtures of these aforementioned polymers can also be used in the present invention. Most preferred polymers from this category include polypropylenes and polystyrenes together with their interpolymers and/or mixtures, because of their cost and mechanical properties.

Illustrative of polyesters which are suitable for use in this invention include those which are derived from the condensation of aromatic, cycloaliphatic, and aliphatic diols with aliphatic, aromatic and cycloaliphatic dicarboxylic acids and may be cycloaliphatic, aliphatic or aromatic polyesters. Exemplary of useful cycloaliphatic, aliphatic and aromatic polyesters which can be utilized in the practice of their invention are poly(ethylene terephthalate), poly(cyclohexenedimethylene), terephthalate) poly(ethylene dodecate), poly(butylene terephthalate), poly(ethylene naphthalate), poly(ethylene(2,7-naphthalate)), poly

(methaphenylene isophthalate), poly(glycolic acid), poly(ethylene succinate), poly(ethylene adipate), poly(ethylene sebacate), poly(decamethylene azelate), poly(ethylene sebacate), poly(decamethylene adipate), poly(decamethylene sebacate), poly(dimethylpropiolactone), poly(para-hydroxybenzoate), poly(ethylene oxybenzoate), poly(ethylene isophthalate), poly(tetramethylene terephthalate), poly(hexamethylene terephthalate), poly(decamethylene terephthalate), poly(1,4-cyclohexane dimethylene terephthalate) (trans), poly(ethylene 1,5-naphthalate), poly(ethylene 2,6-naphthalate), poly(1,4-cyclohexylene dimethylene terephthalate) (cis), and poly(1,4-cyclohexylene dimethylene terephthalate) (trans).

Polyester compounds prepared from the condensation of a diol and an aromatic dicarboxylic acid is preferred for use in this invention. Illustrative of such useful aromatic carboxylic acids are terephthalic acid, isophthalic acid and a *o*-phthalic acid, 1,3-naphthalenedicarboxylic acid, 1,4-naphthalenedicarboxylic acid, 2,6-naphthalenedicarboxylic acid, 2,7-naphthalenedicarboxylic acid, 4,4'-diphenyldicarboxylic acid, 4,4'-diphenylsulfone-dicarboxylic acid, 1,1,3-trimethyl-5-carboxy-3-(*p*-carboxyphenyl)-idane, diphenyl ether 4,4'-dicarboxylic acid, bis-*p*(carboxy-phenyl) methane and the like. Of the aforementioned aromatic dicarboxylic acids, those based on a benzene ring (such as terephthalic acid, isophthalic acid, orthophthalic acid) are preferred for use in the practice of this invention. Amongst these preferred acid precursors, terephthalic acid is particularly preferred acid precursor.

Preferred polyesters for use in the practice of this invention include poly(ethylene terephthalate), poly(butylene terephthalate), poly(1,4-cyclohexylene dimethylene terephthalate) and poly(ethylene naphthalate) and interpolymers and/or mixtures thereof. Among these polyesters of choice, poly(ethylene terephthalate) which may be modified by small amounts of other monomers, is most preferred.

Illustrative of polyamides which are suitable for use in this invention include synthetic linear polycarbonamides characterized by the presence of recurring carbonamide groups as an integral part of the polymer chain, which are separated from one another by at least two carbon atoms. Polyamides of this type include polymers, generally known in the art as nylons, obtained from diamines and dibasic acids having the recurring unit represented by the general formula:



in which R is an alkylene group of at least 2 carbon atoms, preferably from about 2 to about 11 or arylene having at least about 6 carbon atoms, preferably about 6 to about 17 carbon atoms; and R<sup>2</sup> is selected from R<sup>1</sup> and aryl groups. Also, included are copolyamides and terpolyamides obtained by known methods, for example, by condensation of hexamethylene diamine and a mixture of dibasic acids consisting of terephthalic acid and adipic acid. Polyamides of the above description are well-known in the art and include, for example, the copolyamide of 30% hexamethylene diammonium isophthalate and 70% hexamethylene diammonium adipate, poly(hexamethylene adipamide) (nylon 6,6), poly(hexamethylene sebacamide) (nylon 6, 10), poly(hexamethylene isophthalamide), poly(hexamethylene terephthalamide), poly(heptamethylene pimelamide) (nylon 7,7), poly(octamethylene suberamide) (nylon 8,8), poly(nonamethylene azelamide) (nylon 9,9), poly(decamethylene azelamide) (nylon 10,9), poly(decamethylene sebacamide) (nylon 10,10), poly(bis(4-amino cyclohexyl)methane-1,10-

decane-carboxamide)), poly(m-xylylene adipamide), poly(p-xylylene sebacamide), poly(2,2,2-trimethyl hexamethylene terephthalamide), poly(piperazine sebacamide), poly(p-phenylene terephthalamide), poly(metaphenylene isophthalamide) and the like.

Other useful polyamides are those formed by polymerization of amino acids and derivatives thereof, as for example lactams. Illustrative of these useful polyamides are poly(4-aminobutyric acid) (nylon 4), poly(6-aminohexanoic acid) (nylon 6), poly(7-aminohexanoic acid) (nylon 7), poly(8-aminooctanoic acid) (nylon 8), poly(9-aminononanoic acid) (nylon 9), poly(10-amino-decanoic acid) (nylon 10), poly(11-aminoundecanoic acid) (nylon 11), poly(12-aminododecanoic acid) (nylon 12) and the like.

Most preferred polyamides for use in the practice of this invention include poly(caprolactam), poly(12-aminododecanoic acid), poly(hexamethylene adipamide), poly(m-xylylene adipamide), and poly(6-aminohexanoic acid) and interpolymers and/or mixtures thereof.

Illustrative of cellulose esters which are suitable for use in this invention include cellulose nitrate, cellulose triacetate, cellulose diacetate, cellulose acetate propionate, cellulose acetate butyrate, and interpolymers and/or mixtures thereof. Illustrative of a polycarbonate suitable for use in this invention is bisphenol-A polycarbonate. Useful polyvinyl resins include polyvinyl chloride, poly(vinyl acetal) and interpolymers and/or mixtures thereof.

The compatibilizer (component C) of the invention can be any compatibilizer which can ensure compatibility between the polyether polymeric antistat (component A) and the extrudable polymer (component B) by way of controlling phase separation and polymer domain size, so as to provide the desirable Ra of between 0.3  $\mu\text{m}$  and 2.0  $\mu\text{m}$  at the surface. Preferred examples of compatibilizers are: polyethylene, polypropylene, ethylene/propylene copolymers, ethylene/butene copolymers, all these products being grafted with maleic anhydride or glycidyl methacrylate; ethylene/alkyl (meth)acrylate/maleic anhydride copolymers, the maleic anhydride being grafted or copolymerized; ethylene/vinyl acetate/maleic anhydride copolymers, the maleic anhydride being grafted or copolymerized; the two above copolymers in which anhydride is replaced fully or partly by glycidyl methacrylate; ethylene/(meth)acrylic acid copolymers and optionally their salts; ethylene/alkyl (meth)acrylate/glycidyl methacrylate copolymers, the glycidyl methacrylate being grafted or copolymerized, grafted copolymers constituted by at least one mono-amino oligomer of polyamide and of an alpha-mono-olefin (co)polymer grafted with a monomer able to react with the amino functions of said oligomer; Such compatibilizers are described in, among others, EP-A-0,342, 066 and EP-A-0,218,665 which are incorporated herein by reference. Most preferred compatibilizers are terpolymers of ethylene/methyl acrylate/glycidyl methacrylate and copolymers of ethylene/ glycidyl methacrylate, commercially available as Lotader from Elf Atochem or similar products.

The weight ratio of component A: component B can vary between 1:99 to 99:1 but preferably between 15:85 to 85:15, and most preferably between 25:75 and 75:25, to optimize electrical conductivity and mechanical strength. The weight concentration of component C in the mixture of components A, B and C in the layer of the invention can vary between 0.1 to 25%, but preferably between 0.2 to 20% and most preferably between 1 to 15%, to optimize the roughness characteristics and physical properties.

Besides components A, B and C, the present invention may include other optional components. Such optional com-

ponents include nucleating agents, fillers, plasticizers, impact modifiers, chain extenders, colorants, lubricants, antistatic agents, thermally processable onium salts, pigments such as titanium oxide, zinc oxide, talc, calcium carbonate, barium sulfate, clay, etc., dispersants such as fatty amides, (e.g., stearamide), metallic salts of fatty acids, e.g., zinc stearate, magnesium stearate, calcium stearate, etc., dyes such as ultramarine blue, cobalt violet, etc., antioxidants, fluorescent whiteners, ultraviolet absorbers, fire retardants, matte particles or roughening agents, such as silica, titanium dioxide, talc, barium sulfate, clay, and alumina, cross linking agents, voiding agents and the like. These optional components and appropriate amounts are well known in the art and can be chosen according to need.

Of these optional components, thermally processable onium salts, at a level between 0.1-15 weight % of component A, are preferred. Also preferred are pigments and particles, such as those selected from the group consisting of silica, titanium dioxide, talc, barium sulfate, clay, and alumina, with a preferred particle size in the range of 0.2  $\mu\text{m}$  to 10  $\mu\text{m}$ . Such a particle size range is chosen to optimize the desired surface effect without creating unwanted surface voids during the biaxial orientation process or embossing the front surface when the material is tightly wound in a roll.

The web of the invention can comprise a single layer or multiple layers according to need. The multiplicity of layers may include any number of auxiliary layers such as anti-static layers, backmark retention layers, tie layers or adhesion promoting layers, abrasion resistant layers, conveyance layers, barrier layers, splice providing layers, UV absorption layers, antihalation layers, optical effect providing layers, waterproofing layers, flavor retaining layers, fragrance providing layers, adhesive layers, imaging layers and the like.

The web of the invention can be formed by any method known in the art such as those involving extrusion, coextrusion, quenching, orientation, heat setting, lamination, etc. It is preferred that the web of the invention is an oriented sheet formed by any suitable method known in the art, such as by a flat sheet process or a bubble or tubular process. The flat sheet process involves extruding or coextruding the materials of the sheet through a slit die and rapidly quenching the extruded or coextruded web upon a chilled casting drum so that the polymeric component(s) of the sheet are quenched below their solidification temperature. The quenched sheet is then biaxially oriented by stretching in mutually perpendicular directions at a temperature above the glass transition temperature of the polymer(s). The sheet may be stretched in one direction and then in a second direction or may be simultaneously stretched in both directions. The preferred stretch ratio in any direction is at least 3:1. After the sheet has been stretched, it is heat set by heating to a temperature sufficient to crystallize the polymers while restraining to some degree the sheet against retraction in both directions of stretching.

The web of the invention may be subjected to any number of coatings and treatments, after extrusion, coextrusion, orientation, etc. or between casting and full orientation, to improve its properties, such as printability, barrier properties, heat-sealability, spliceability, adhesion to other supports and/or imaging layers. Examples of such coatings can be acrylic coatings for printability, polyvinylidene halide for heat seal properties, etc. Examples of such treatments can be flame, plasma and corona discharge treatment, to improve printability and adhesion. Further examples of treatments can be calendaring, embossing, patterning, etc. to obtain specific effects on the surface of the web. The web of the invention can be incorporated in any other suitable

support by lamination, extrusion coating, or any other method known in the art.

The surface roughness of the web or Ra is a measure of relatively finely spaced surface irregularities such as those produced on the backside of photographic materials by the casting of polyethylene against a rough chilled roll. The surface roughness measurement is a measure of the maximum allowable roughness height expressed in units of micrometers and by use of the symbol Ra. For the irregular profile of the backside of photographic materials of this invention, the average peak to valley height, which is the average of the vertical distances between the elevation of the highest peak and that of the lowest valley, is used.

Biaxially oriented sheets commonly used in the packaging industry are commonly melt extruded and then orientated in both directions (machine direction and cross direction) to give the sheet desired mechanical strength properties. The process of biaxial orientation generally creates a surface roughness of less than 0.2  $\mu\text{m}$ . While the smooth surface may have value in the packaging industry, use as a backside layer for photographic paper is limited. Laminated to the backside of the base paper, the biaxially oriented sheet must have a surface roughness greater than 0.30  $\mu\text{m}$  to ensure efficient transport through the many types of photofinishing equipment that have been purchased and installed around the world. At surface roughness less than 0.30  $\mu\text{m}$ , transport through the photofinishing equipment becomes less efficient. At surface roughness greater than 2.54  $\mu\text{m}$ , the surface would become too rough causing transport problems in photofinishing equipment, and the rough backside surface would begin to emboss the silver halide emulsion as the material is wound in rolls.

A preferred application of the web of the invention is in imaging elements, including those utilizing photographic, electrophotographic, electrostagraphic, photothermographic, migration, electrothermographic, dielectric recording, thermal dye transfer, ink jet and other types of imaging. A more preferred application of the web of the invention is in photographic imaging elements, particularly photographic paper and other display products.

Typical imaging supports comprise cellulose nitrate, cellulose acetate, poly(vinyl acetate), polystyrene, polyolefins, poly(ethylene terephthalate), poly(ethylene naphthalate), polycarbonate, polyamide, polyimide, glass, natural and synthetic paper, resin-coated paper, voided polymers including polymeric foam, microvoided polymers and microporous materials, fabric, etc., and the web of this invention can be incorporated in any suitable support. The material can be placed anywhere in the imaging support, e.g., on the top side, or the bottom side, or both sides. However, it is preferred to be placed on the bottom side of the imaging support.

The web of this invention provides a surface roughness Ra of between 0.3  $\mu\text{m}$  and 2.0  $\mu\text{m}$ , and preferably between 0.4-4  $\mu\text{m}$  and 1.5  $\mu\text{m}$ . The coefficient of friction (COF) for such a web is less than 0.4, and preferably less than 0.3 to ensure smooth transport with minimal dusting. The surface electrical resistivity or SER of the web of this invention is 13 log ohms/square or less, and preferably 12.5 log ohms/square or less, before and after any wet photographic processing. In a preferred embodiment, the imaging material of this invention is incorporated in imaging supports used for image display such as papers, particularly resin-coated papers, voided polymers, and combinations thereof. Particularly suited for the application of the present invention are imaging supports disclosed in U.S. Pat. Nos. 3,411,908; 3,501,298; 4,042,398; 4,188,220; 4,699,874; 4,794,071;

4,801,509; 5,244,861; 5,326,624; 5,395,689; 5,466,519; 5,780,213; 5,853,965; 5,866,282; 5,874,205; 5,888,643; 5,888,681; 5,888,683; 5,902,720; 5,935,690; 5,955,239; 5,994,045; 6,017,685; 6,017,686; 6,020,116; 6,022,677; 6,030,742; 6,030,756; 6,030,759; 6,040,036; 6,043,009; 6,045,965; 6,063,552; 6,071,654; 6,071,680; 6,074,788; 6,074,793; and incorporated herein by reference.

In one preferred embodiment of the invention for application in photographic display product, a biaxially oriented web of this invention with the skin layer on the bottom of the photographic element is formed with the following structure:

Solid core containing one or more layers

Skin layer

The solid core and the skin layer may be cast by co-extrusion followed by preheating, orientation, and heat setting as a preferred method. The web of the invention may or may not be voided. The skin layer comprises components A, B and C of the invention in appropriate amounts, and therefore is of the desired roughness and antistatic characteristics. The solid core may comprise any extrudable polymer, such as those described for component B of the invention. It is preferred that the solid core comprises the same thermoplastic polymer as the one chosen for component B in the skin layer, for better adhesion. Alternatively, if the skin and the core comprise different thermoplastic polymers, adhesion may be improved through the use of a tie layer or a suitable adhesion promoting agent. As described herein above, the web of the invention can comprise any optional addenda in any amount, any number of auxiliary layers, and can be subjected to any coatings or treatments to fulfill specific needs of the application. The thickness of the preferred biaxially oriented web can vary between 10  $\mu\text{m}$  to 150  $\mu\text{m}$ . Below 15  $\mu\text{m}$ , the web may not be thick enough to minimize any inherent non-planarity in the support and would be more difficult to manufacture. At thickness higher than 70  $\mu\text{m}$ , little improvement in physical properties can be obtained to justify further increase in cost for extra materials. The thickness of the skin layer relative to the total thickness of the web (i.e., core plus skin thickness) can be of any value but is preferred to be between 0.1% to 25% of the total thickness, and more preferably between 1% and 20% of the total thickness.

In this preferred embodiment, the web of the invention is incorporated on to the backside of a photographic display type support, which could comprise paper, synthetic paper, voided polymers including microvoided polyethylene terephthalate such as those disclosed in U.S. Pat. Nos. 4,912,333; 4,994,312; and 5,055,371; microvoided polyolefins such as those disclosed in U.S. Pat. Nos. 5,244,861; 5,352,653 and 6,071,654; and microporous materials such as those disclosed in U.S. Pat. Nos. 4,833,172; 4,861,644; 4,877,679; 4,892,779; 4,972,802; 4,937,115; 4,957,787; 4,959,208; 5,032,450; 5,035,886; 5,047,283; 5,071,645; 5,114,438; 5,196,262; 5,326,391 and 5,583,171; cloth, woven polymer fibers, or combinations thereof. In the most preferred embodiment for photographic display, the web of the invention is adhered to the backside of photographic paper base comprising natural cellulosic paper fibers.

When using a cellulose fiber paper support, it is preferable to extrusion laminate the web of the invention to the base paper using a polyolefin resin. Extrusion laminating is carried out by bringing together the biaxially oriented web of the invention and the base paper with application of an adhesive between them followed by their being pressed in a nip such as between two rollers. The adhesive may be applied to either the biaxially oriented web or the base paper

prior to their being brought into the nip. In a preferred form the adhesive is applied into the nip simultaneously with the biaxially oriented web and the base paper. The adhesive may be any suitable material that does not have a harmful effect upon the photographic element. A preferred material is polyethylene that is melted at the time it is placed into the nip between the paper and the biaxially oriented sheet.

During the lamination process, it is desirable to maintain control of the tension of the biaxially oriented web in order to minimize curl in the resulting laminated support. For high humidity applications (>50% RH) and low humidity applications (<20% RH), it is desirable to laminate both a front side and backside film to keep curl to a minimum.

The front side film can be any polymer based film, which may comprise voided polymers including microvoided polymers and microporous materials, such as referenced herein before. Particularly suitable front side films, preferred methods of their formation and application to imaging supports such as photographic display products are disclosed in U.S. Pat. Nos. 5,853,965; 5,866,282; 5,874,205; 5888,643; 5,902,720; 5,994,045; etc. and references therein.

In one preferred embodiment, in order to produce photographic elements with a desirable photographic look and feel, it is preferable to use relatively thick paper supports, e.g., at least 120  $\mu\text{m}$  thick, preferably from 120  $\mu\text{m}$  to 250  $\mu\text{m}$  thick, and relatively thin front side films comprising microvoided composite sheets e.g., less than 50  $\mu\text{m}$  thick, preferably from 20  $\mu\text{m}$  to 50  $\mu\text{m}$  thick, more preferably from 30  $\mu\text{m}$  to 50  $\mu\text{m}$  thick.

The preferred photographic element is a material that utilizes photosensitive silver halide in the formation of images. In the case of thermal dye transfer or ink jet, the image layer that is coated on the imaging element may be any material that is known in the art such as gelatin, pigmented latex, polyvinyl alcohol, polycarbonate, polyvinyl pyrrolidone, starch, and methacrylate. The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

The photographic emulsions useful for this invention are generally prepared by precipitating silver halide crystals in a colloidal matrix by methods conventional in the art. The colloid is typically a hydrophilic film forming agent such as gelatin, alginic acid, or derivatives thereof

The crystals formed in the precipitation step are washed and then chemically and spectrally sensitized by adding spectral sensitizing dyes and chemical sensitizers, and by providing a heating step during which the emulsion temperature is raised, typically from 40.degree. C. to 70.degree. C., and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sen-

sitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, curtain coating and extrusion coating.

The silver halide emulsions utilized in this invention may be comprised of any halide distribution. Thus, they may be comprised of silver chloride, silver chloroiodide, silver bromide, silver bromochloride, silver chlorobromide, silver iodochloride, silver iodoform, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride; and optimally greater than about 95 mole percent silver chloride.

The silver halide emulsions can contain grains of any size and morphology. Thus, the grains may take the form of cubes, octahedrons, cubo-octahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H. James, Macmillan Publishing Company, Inc., 1977, pages 151-152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitization include ascorbic acid derivatives; tin compounds; polyamine compounds; and thiourea dioxide-based compounds described in U.S. Pat. Nos. 2,487,850; 2,512,925; and British Patent 789,823. Specific examples of reduction sensitizers or conditions, such as dimethylamineborane, stannous chloride, hydrazine, high pH (pH 8-11) and low pAg (pAg 1-7) ripening are discussed by S. Collier in *Photographic Science and Engineering*, 23,113 (1979). Examples of processes for preparing intentionally reduction sensitized silver halide emulsions are described in EP 0 348934 A1 (Yamashita), EP 0 369491 (Yamashita), EP 0 371388 (Ohashi), EP 0 396424 A1 (Takada), EP 0 404142 A1 (Yamada), and EP 0 435355 A1 (Makino).

The photographic elements of this invention may use emulsions doped with Group VIII metals such as iridium, rhodium, osmium, and iron as described in Research

Disclosure, September 1996, Item 38957, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," Photographic Science and Engineering, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in The British Journal of Photography Annual, 1982, pages 201-203.

A typical multicolor photographic element of the invention comprises the invention laminated support bearing a cyan dye image-forming unit comprising at least one red-sensitive silver halide emulsion layer having associated therewith at least one cyan dye-forming coupler, a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black and white photographic print elements.

The photographic elements may also contain a transparent magnetic recording layer such as a layer containing magnetic particles on the underside of a transparent support, as in U.S. Pat. Nos. 4,279,945 and 4,302,523. Typically, the element will have a total thickness (excluding the support) of from about 5 to about 30  $\mu$ m.

In the following table, reference will be made to (1) Research Disclosure, December 1978, Item 17643, (2) Research Disclosure, December 1989, Item 308119, and (3) Research Disclosure, September 1996, Item 38957, all published by Kenneth Mason Publications, Ltd., Dudley Annex, 12a North Street, Emsworth, Hampshire PO10 7DQ, ENGLAND. The table and the references cited in the table are to be read as describing particular components suitable for use in the elements of the invention. The table and its cited references also describe suitable ways of preparing, exposing, processing and manipulating the elements, and the images contained therein.

-continued

| Reference Section | Subject Matter                            |
|-------------------|-------------------------------------------|
| 5                 | VI                                        |
| 2                 | VII                                       |
| 3                 | VIII Absorbing and scattering             |
| 1                 | VIII, XIII, materials; Antistatic layers; |
| 2                 | XVI matting agents                        |
| 3                 | VIII, IX C                                |
| 10                | & D                                       |
| 1                 | VII Image-couplers and image-             |
| 2                 | VII modifying couplers, Dye               |
| 3                 | X stabilizers and hue modifiers           |
| 1                 | XVII Supports                             |
| 2                 | XVII                                      |
| 3                 | XV                                        |
| 3                 | XI Specific layer arrangements            |
| 3                 | XII, XIII Negative working emulsions;     |
| 25                | Direct positive emulsions                 |
| 2                 | XVIII Exposure                            |
| 3                 | XVI                                       |
| 1                 | XIX, XX Chemical processing;              |
| 2                 | XIX, XX Developing agents                 |
| 30                | XXII                                      |
| 3                 | XVIII, XIX,                               |
| 3                 | XX                                        |
| 25                | XIV Scanning and digital                  |
|                   | processing procedures                     |

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible image, preferably by other than heat treatment. Processing is preferably carried out in the known RA-4.TM. (Eastman Kodak Company) Process or other processing systems suitable for developing high chloride emulsions.

The laminated substrate of the invention may have copy restriction features incorporated such as disclosed in U.S. patent application Ser. No. 08/598,785 filed Feb. 8, 1996 and application Ser. No. 08/598,778 filed on the same day. These applications disclose rendering a document copy restrictive by embedding into the document a pattern of invisible microdots. These microdots are, however, detectable by the

50 electro-optical scanning device of a digital document copier. The pattern of microdots may be incorporated throughout the document. Such documents may also have colored edges or an invisible microdot pattern on the backside to enable users or machines to read and identify the media. The media 55 may take the form of sheets that are capable of bearing an image. Typical of such materials are photographic paper and film materials composed of polyolefin resin coated paper, polyester, (poly)ethylene naphthalate, and cellulose triacetate based materials.

60 The microdots can take any regular or irregular shape with a size smaller than the maximum size at which individual microdots are perceived sufficiently to decrease the usefulness of the image, and the minimum level is defined by the detection level of the scanning device. The microdots 65 may be distributed in a regular or irregular array with center-to-center spacing controlled to avoid increases in document density. The microdots can be of any hue,

| Reference Section | Subject Matter                               |
|-------------------|----------------------------------------------|
| 1                 | I, II Grain composition,                     |
| 2                 | I, II, IX, X,<br>morphology and preparation. |
| 3                 | XI, XII, Emulsion preparation                |
| 1                 | XIV, XV including hardeners, coating         |
| 2                 | I, II, III, IX<br>aids, addenda, etc.        |
| 3                 | A & B                                        |
| 1                 | III, IV Chemical sensitization and           |
| 2                 | III, IV spectral sensitization/              |
| 3                 | IV, V desensitization                        |
| 1                 | V UV dyes, optical brighteners,              |
| 2                 | V luminescent dyes                           |
| 3                 | VI                                           |
| 1                 | VI Antifoggants and stabilizers              |

brightness, and saturation that does not lead to sufficient detection by casual observation, but preferably of a hue least resolvable by the human eye, yet suitable to conform to the sensitivities of the document scanning device for optimal detection.

In one embodiment the information-bearing document is comprised of a support, an image-forming layer coated on the support and pattern of microdots positioned between the support and the image-forming layer to provide a copy restrictive medium. Incorporation of the microdot pattern into the document medium can be achieved by various printing technologies either before or after production of the original document. The microdots can be composed of any colored substance, although depending on the nature of the document, the colorants may be translucent, transparent, or opaque. It is preferred to locate the microdot pattern on the support layer prior to application of the protective layer, unless the protective layer contains light scattering pigments. Then the microdots should be located above such layers and preferably coated with a protective layer. The microdots can be composed of colorants chosen from image dyes and filter dyes known in the photographic art and dispersed in a binder or carrier used for printing inks or light-sensitive media.

In a preferred embodiment the creation of the microdot pattern as a latent image is possible through appropriate temporal, spatial and spectral exposure of the photosensitive materials to visible or non-visible wavelengths of electromagnetic radiation. The latent image microdot pattern can be rendered detectable by employing standard photographic chemical processing. The microdots are particularly useful for both color and black-and-white image-forming photographic media. Such photographic media will contain at least one silver halide radiation sensitive layer, although typically such photographic media contain at least three silver halide radiation sensitive layers. It is also possible that such media contain more than one layer sensitive to the same region of radiation. The arrangement of the layers may take any of the forms known to one skilled in the art, as discussed in Research Disclosure 37038 of February 1995.

The following examples illustrate the practice of this invention. They are not intended to be exhaustive of all possible variations of the invention. Parts and percentages are by weight unless otherwise indicated.

#### EXAMPLES

Examples of biaxially oriented webs of this invention are prepared with a skin layer comprising components A, B and C, on a solid core of polypropylene as schematically shown below:

Solid core containing polypropylene

Skin layer containing components A, B and C

Component A in the skin layer is chosen to be Pebax MV 1074, a polyether-block-copolyamide, supplied by Elf Atochem. Pebax MV 1074 is a polyamide-12 based polymer with a PEG ether segment. Component B in the skin layer is chosen to be P4G2Z-073A, a homopolymer of polypropylene, supplied by Huntsman, for samples Ex. 1-4, and a low density polyethylene Tenite PE D4002-P, supplied by Eastman Chemicals, for Ex. 5. Component C in the skin layer is Lotader 8900, a terpolymer of ethylene/methyl acrylate/glycidyl methacrylate, also supplied by Elf Atochem. The polypropylene of the solid core is the same as component B in the skin layer of Ex. 1-4.

The material of the skin layer, with varying ratios of components A, B and C, is pre-compounded and pelletized in a co-rotating twin screw compounder. The pellets of the

precompounded material for the skin and the polypropylene for the core, are dried at 65° C. and fed by two plasticating screw extruders into a co-extrusion die manifold to produce a two-layered melt stream, which is rapidly quenched on a 5 chill roll after issuing from the die. By regulating the throughputs of the extruders it is possible to adjust the thickness ratio of the skin layer and the core in the cast sheet. In these cast sheets, the core layer thickness is nominally maintained at 750  $\mu\text{m}$ . The cast sheet thus formed is 10 stretched in the machine direction by 5x and in the transverse direction in a tenter frame by another 5x, at a temperature of 150° C. to form a sample sheet, wherein the core thickness is approximately 30  $\mu\text{m}$ .

For resistivity tests, samples are preconditioned at 15% RH (unless otherwise noted) and at 72° F. for at least 24 hours prior to testing. Surface electrical resistivity (SER) of the skin layer is measured with a Keithly Model 616 digital electrometer using a two point DC probe by a method similar to that described in U.S. Pat. No. 2,801,191. SER can be measured before and after the sample has been run though a typical wet chemical processing, such as C-41 processing. For desirable performance, the antistatic skin layer should exhibit SER values <13 log ohms/square.

For backmark retention (BMR) tests, a printed image is 25 applied onto the skin layer of the ample using a dot matrix printer. The sample is then subjected to a conventional developer for 30 seconds, washed with warm water for 5 seconds and rubbed for print retention evaluation. The following ratings are assigned,

30 1=Outstanding, very little difference between processed and unprocessed appearance.  
2=Excellent, slight degradation of appearance  
3=Acceptable, medium degradation of appearance  
4=Unacceptable, serious degradation of appearance  
5=Unacceptable, total degradation.

For desirable performance, the BMR rating should be <4. For roughness or Ra values a Gould Microtopographer stylus instrument is used, utilizing a diamond stylus with a 40 light load of 50 mg to avoid surface damage. The roughness average Ra of the skin layer is determined, as per ASME B46.1-1995. The roughness average, Ra is the arithmetic average of the absolute values of the profile height deviations recorded within the evaluation length and measured 45 from the mean line. Ra values are expressed in  $\mu\text{m}$ .

For writability, an ordinary pencil is used to write indicia on the skin layer of the sample. Dark, clearly legible indicia indicate "good" writability of the sample.

Working examples, Ex. 1-5, are prepared, as per the 50 invention, utilizing components A, B and C in varying ratios in the skin layer with different thickness, on a polypropylene core. Ex. 1-4 utilize polypropylene (PP) as component B in the skin layer whereas Ex. 5 utilize a low density polyethylene (PE) as component B in the skin layer.

55 Comparative samples, Comp. 1-2, are prepared similar to Ex. 1 and 3, except without component C. Comparative sample Comp. 3 is just a solid polypropylene film without the skin layer of the invention. Comparative sample Comp. 4 is a commercially available film, BICOR 70 MLT, supplied by Mobil Chemical Co., disclosed to be illustrative of the teaching of U.S. Pat. No. 6,022,677. Comparative sample, Comp. 5, is the same as Comp. 4 but coated over the skin layer with an antistatic layer comprising colloidal silica, polymerized alkylene oxide and alkali metal salt as the conductive agent, and a styrene acrylate film forming binder. Such an antistatic layer is typical of the art for photographic paper antistats, as illustrated in U.S. Pat. No. 5,244,728.

Details of these samples are listed in Table 1, and the appearance and physical properties of these samples determined as per tests described herein above, are listed in Table 2.

TABLE 1

| Sample | Skin layer                                          |          |                                   |                          |                             |          |
|--------|-----------------------------------------------------|----------|-----------------------------------|--------------------------|-----------------------------|----------|
|        | Component A<br>Pebax MV                             | Weight % | Component B<br>Polypropylene (PE) | Weight %                 | Component C<br>Lotader 8900 | Weight % |
| Ex.1   | 50                                                  | 40 (PP)  | 10                                | 100                      | 4                           | 30       |
| Ex.2   | 50                                                  | 40 (PP)  | 10                                | 100                      | 0.8                         | 30       |
| Ex.3   | 30                                                  | 60 (PP)  | 10                                | 100                      | 4                           | 30       |
| Ex.4   | 30                                                  | 60 (PP)  | 10                                | 100                      | 0.8                         | 30       |
| Ex.5   | 30                                                  | 60 (PE)  | 10                                | 100                      | 4                           | 30       |
| Comp.1 | 50                                                  | 50       | 0                                 | 100                      | 4                           | 30       |
| Comp.2 | 30                                                  | 70       | 0                                 | 100                      | 4                           | 30       |
| Comp.3 | 0                                                   | 0        | 0                                 | 100                      | 0                           | 30       |
| Sample | Skin layer composition                              |          |                                   | Core layer composition   |                             |          |
| Comp.4 | Block copolymer of polyethylene and polypropylene   |          |                                   | Solid polypropylene core |                             |          |
| Comp.5 | Same as Comp.4 but coated with an antistatic layer. |          |                                   | Same as Comp.4           |                             |          |

TABLE 2

| Sample | appear-<br>ance                    | Pre<br>C-41<br>SER<br>log<br>ohms/<br>square | Post<br>C-41<br>SER<br>log<br>ohms/<br>square | Rough-<br>ness<br>Ra | Writ-<br>ability | BMR | COF |
|--------|------------------------------------|----------------------------------------------|-----------------------------------------------|----------------------|------------------|-----|-----|
|        |                                    |                                              |                                               |                      |                  |     |     |
| Ex.1   | Trans-<br>lucent<br>smooth         | 11.4                                         | 10.9                                          | 1.42                 | good             | 2   | 0.2 |
| Ex.2   | Trans-<br>lucent<br>smooth         | 12.4                                         |                                               |                      | good             |     |     |
| Ex.3   | Trans-<br>lucent<br>smooth         | 11.4                                         | 11.1                                          | 1.09                 | good             | 2-3 | 0.2 |
| Ex.4   | Trans-<br>lucent<br>smooth         | 12.2                                         |                                               |                      | good             |     |     |
| Ex.5   | Trans-<br>lucent<br>smooth         | 11.4                                         |                                               | 1.52                 | good             | 2-3 | 0.2 |
| Comp.1 | Milky<br>Very<br>rough             | 11.4                                         |                                               | 6.16                 | good             |     |     |
| Comp.2 | Milky<br>Very<br>rough             | 12.1                                         |                                               | 4.33                 | good             |     |     |
| Comp.3 | Trans-<br>parent<br>Very<br>smooth | >13                                          | >13                                           | 0.13                 | none             | 4-5 |     |
| Comp.4 | Trans-<br>lucent<br>smooth         | >13                                          | >13                                           | 0.47                 | good             | 3-4 |     |
| Comp.5 | Trans-<br>lucent<br>smooth         | 11.8                                         | >13                                           |                      | good             | 2-3 |     |

It is obvious from Table 2 that samples Ex. 1-5, prepared in accordance with this invention, provide antistatic characteristics, as reflected by SER <13 log ohms/square, as well as the desired roughness, as reflected by Ra between 0.3  $\mu\text{m}$  and 2  $\mu\text{m}$ . Ex. 1 and 3 also demonstrate low SER (<13 log ohms/square) after C-41 processing, illustrating their antistatic characteristics even after a wet chemical processing. This indicates that if these webs are incorporated in photographic paper, they are less likely to face post-processing print sticking from static charge generation. The examples of the invention also demonstrate good writability and backside printability (as reflected by a BMR rating of <4), two highly desirable characteristics for display type applications of the web of the invention. The coefficient of friction (COF) for the examples of this invention is also desirably <0.3, ensuring smooth transport of the web during manufacturing and subsequent use.

Comparative samples, Comp. 1 and 2, which are prepared similar to Ex. 1 and 3, respectively, but without component C, reveal a milky white coating with very high degree of surface roughness of Ra >4. Such high roughness is undesirable as it can cause embossing of the image layer when tightly wound in a roll form as an imaging element. Because of such high roughness, it is also likely to cause difficulty during transport and possible dusting as the asperities from the rough layer rub against conveyance rollers and other surfaces.

Comparative sample, Comp.3, prepared with just polypropylene without the skin layer of the invention, is neither antistatic nor sufficiently rough, to afford writability and ease of conveyance.

Comparative Sample, Comp.4, illustrative of the roughening layer of U.S. Pat. No. 6,022,677, is desirably rough and writable but not conductive enough (SER >13 log ohms/square) to provide necessary static protection. Such a sheet needs to be additionally coated with an antistat, as in comparative sample Comp.5, to have the necessary conductivity (SER <13 log ohms/square). However, even with that additional coating of an antistat, Comp.5 loses its conductivity after wet chemical processing (SER >13 log ohms/square), and thus may be vulnerable to print sticking and other problems after photofinishing.

The invention has been described in detail with particular reference to certain preferred embodiments thereof, but it will be understood that variations and modifications can be effected within the spirit and scope of the invention.

What is claimed is:

- An imaging member comprising an imaging layer and a substrate wherein said substrate comprises at least one surface layer comprising polyether polymeric antistat, extrudable polymer, and compatibilizer wherein said surface layer has a roughness of greater than 0.3 Ra.
- The imaging member of claim 1 wherein said surface layer is on the bottom of said imaging material and is the lower surface layer of an oriented polymer sheet.
- The imaging member of claim 2 wherein said oriented polymer sheet comprises a biaxially oriented polyolefin sheet.
- The imaging member of claim 2 wherein said oriented polymer sheet has been stretched in at least one direction to a length three times its original dimension.
- The imaging member of claim 1 wherein said surface layer has a resistivity of less than 13 log ohm/sq.
- The imaging member of claim 1 wherein said polyether polymeric antistat comprises polyether block copolyamide.
- The imaging member of claim 1 wherein said extrudable polymer comprises polypropylene.

**21**

8. The imaging member of claim 1 wherein said extrudable polymer comprises polyethylene.

9. The imaging member of claim 1 wherein said extrudable polymer comprises polyolefin terpolymer.

10. The imaging member of claim 1 wherein said extrudable polymer comprises polyester.

11. The imaging member of claim 1 wherein said roughness is between 0.3 Ra and 2 Ra.

12. The imaging member of claim 1 wherein said resistivity is less than 12.5 log ohm/sq.

13. The imaging member of claim 1 wherein said polyether polymeric antistat comprises between 15 and 85% weight by layer, said extrudable polymer comprises between 15 and 85% by weight of said layer, and said compatibilizer comprises between 0.2 and 20% by weight of said layer.

14. The imaging member of claim 1 further comprising slip additives.

15. The imaging member of claim 1 wherein said surface layer has a coefficient of friction of less than 0.3.

16. The imaging member of claim 1 wherein said surface layer comprises particles having a size range between 0.2  $\mu\text{m}$  and 10  $\mu\text{m}$ .

17. The imaging member of claim 1 wherein said particles are selected from the group consisting of silica, titanium dioxide, talc, barium sulfate, clay, and alumina.

18. An imaging member comprising an imaging layer and a substrate wherein said substrate comprises at least one surface layer comprising polyether polymeric antistat, extrudable polymer, and compatibilizer wherein said surface layer has a roughness of greater than 0.3 Ra, and wherein said imaging member comprises thermally processable onium salt.

19. The imaging member of claim 18 wherein said thermally processable onium salt comprises between 0.1 and 10% by weight of the amount of said polyether polymeric antistat.

20. The imaging member of claim 1 wherein said compatibilizer comprises at least one member selected from the

**22**

group consisting of polyethylene, polypropylene, ethylene/propylene copolymers, ethylene/butene copolymers, polyethylene, polypropylene, ethylene/propylene copolymers, ethylene/butene copolymers grafted with maleic anhydride or glycidyl methacrylate, ethylene/alkyl (meth)acrylate/maleic anhydride copolymers wherein the maleic anhydride is grafted or copolymerized, ethylene/vinyl acetate/maleic anhydride copolymers wherein the maleic anhydride is grafted or copolymerized, ethylene/alkyl (meth)acrylate/maleic anhydride copolymers and ethylene/vinyl acetate/maleic anhydride copolymers wherein anhydride is replaced fully or partly by glycidyl methacrylate, ethylene/(meth)acrylic acid copolymers and their salts, ethylene/alkyl (meth)acrylate/glycidyl methacrylate copolymers wherein the glycidyl methacrylate is grafted or copolymerized, and grafted copolymers constituted by at least one mono-amino oligomer of polyamide and of an alpha-mono-olefin (co)polymer grafted with a monomer able to react with the amino functions of said oligomer.

21. The imaging member of claim 1 wherein said compatibilizer comprises at least one member selected from the group consisting of polyethylene, polypropylene, ethylene/propylene copolymers, ethylene/butene copolymers, polyethylene, polypropylene, ethylene/propylene copolymers, ethylene/butene copolymers grafted with maleic anhydride or glycidyl methacrylate, ethylene/alkyl (meth)acrylate/maleic anhydride copolymers, ethylene/vinyl acetate/maleic anhydride copolymers, ethylene/alkyl (meth)acrylate/glycidyl methacrylate copolymers, and ethylene/glycidyl methacrylate.

22. The imaging member of claim 1 wherein said compatibilizer comprises terpolymers of ethylene/methyl acrylate/glycidyl methacrylate or copolymers of ethylene/glycidyl methacrylate.

\* \* \* \* \*